

Dec. 4, 1956

G. G. OBERFELL

2,772,634

SHOTGUN CARTRIDGE AND SHOT FOR THE SAME

Filed Feb. 16, 1950



FIG. 1



FIG. 2

INVENTOR.  
G. G. OBERFELL

BY *Hudson & Young*

ATTORNEYS

1

2,772,634

**SHOTGUN CARTRIDGE AND SHOT FOR THE SAME**

George G. Oberfell, Bartlesville, Okla.

Application February 16, 1950, Serial No. 144,588

4 Claims. (Cl. 102—42)

This invention relates to shotgun cartridges and to shot for shotgun cartridges. Such shot are frequently referred to as pellets, and such cartridges are well-known in the trade as shotgun shells or shot shells. In one aspect, this invention relates to shot for shotgun cartridges, said shot being surface-treated with a substance for the purpose of imparting a thin film of lubricating material to the individual pellets which makes them non-adherent and prevents metal to metal contact between said pellets. In another aspect, this invention relates to metallic pellets for shotgun shells, said pellets coated with a thin film which inhibits oxidation of the metal of the pellets due to reducing the amount of contact between the metal and the surrounding air and due to the inhibiting or lessening of the oxidation reactions. In another aspect, this invention relates to a process for reducing the tendency of shot to cling together when being fired from a shotgun, which tendency results in undesirable large concentration of the shot at certain points in the distribution pattern with a resulting increase in void spaces in said pattern, known as patches, which are of sufficient diameter to allow a game bird, or other animal, occupying the position of said patch to escape being killed by said shot, or a clay target to pass on unbroken.

I have found from a study of several hundred targets that the pattern of ordinary shot charges fired at targets shows a more uneven distribution of pellet holes in the target than would be experienced if the pellets were free to travel completely independent of each other after passing the muzzle of the shotgun after it is fired. In localized areas of the shot pattern, there are concentrations of shot in the form of close groups or clusters of two or more shot, whereas in other areas there are very few shot or none at all. I have found that this tendency for shot to concentrate in groups is due in turn to the tendency of the pellets to adhere to each other, or to stick together, due to metal to metal contact of the pellets. As the shot charge is forced under high pressure through the various portions of the bore of the shotgun, particularly through the constricted portion which is known as the "choke," a balling or welding effect takes place which makes the pellets tend to cling to each other. However, even in true cylinder bores, the force of the explosion of the powder drives the shot into metal to metal contact with sufficient force to cause some of the shot to cling together enough to increase the patches in the pattern. This tendency of the pellets to cling to each other is aggravated when the shot is old and has had time to become more or less corroded or oxidized. In passing through the air toward the target the air resistance may actually separate the pellets, but they will still be too close together to give a good pattern due to having adhered to each other for a period of time.

I have found that by surface-treating the pellets of the shot charge which is loaded into the shotgun cartridge with suitable materials in order to impart a thin layer

2

or film of lubricating material on the pellets, rendering them non-adherent, thereby preventing metal to metal contact of pellets as they pass through the shotgun bore, I materially reduce the number of patches or voids of substantial diameter in the shot pattern and obtain more even distribution of the pellets through the pattern. It is preferable that the material used for surface-treating of the pellets be of an oxidation preventing, reducing, or inhibiting nature.

One object of the present invention is to reduce and substantially eliminate the balling, welding, or clinging or sticking together of the shot in the shot charge during its passage through the bore of the shotgun when the gun is fired.

Another object is to produce an improved shotgun cartridge and shot for the same.

Another object is to inhibit or reduce the amount of oxidation of metallic shot in shotgun charges in order to reduce the tendency of the shot to adhere or cling together.

Another object is to reduce the number of patches or void spaces of large diameter in the pattern of shot from the shotgun, and to produce a more even distribution of shot in the shotgun pattern by reducing the tendency of the shot to concentrate in groups in some areas, particularly in the center of the shotgun pattern.

A number of other objects and advantages will be apparent to those skilled in the art upon reading the specification and claims of this invention.

In the drawings:

Figure 1 is an elevational cross-sectional view of a shotgun loaded with a shotgun shell containing shot coated in accordance with the present invention.

Figure 2 is an enlarged cross-sectional elevational view of one of the coated shot pellets shown in Figure 1.

Figure 1 is based on the disclosure in Figure 1 of my copending application Serial No. 146,558, filed February 27, 1950, now U. S. Patent 2,658,298 of November 10, 1953, except that a conventional prior art choke 32 is shown in the present application, and shot 23 are coated with the materials set forth only in the present specification as a coating 30 shown only in Figure 2 of the present application, of which figure there is no counterpart in my said copending application.

In Figure 1, a conventional shotgun of the prior art generally designated as 7 is provided with a choke section generally designated as 8. The shotgun has a generally cylindrical gun barrel 9, the internal diameter of which decreases in passing out the muzzle through the conical or otherwise tapered choke section 32.

The shotgun 7 is entirely conventional. It consists of a barrel 9 having one end sealed by breach block 12 which contains a firing mechanism (not shown) which may comprise a hammer 13. A conventional shot gun shell 14 comprises a base 16, having a percussion cap, or primer 17, powder charge 18, powder chamber 19, wads 20, 21 and 22, shot pellets 23 which are conventional except that they are coated with a coating 30 (Figure 2) as will be described later, front wad 24 and container 26. Container 26 is either crimped at 27 to retain front wad 24, or 27 is folded in some manner (not shown) in front of shot 23, in which case front wad 24 may be eliminated.

Shotgun barrel 9 has a bore comprising a chamber 28, a connecting conical portion 29, a substantially cylindrical bore 31, and a choke section 8.

In Figure 2, one of the shot 23 of Figure 1 is shown enlarged about twenty-five diameters and in cross-section. The conventional lead shot 25 has a plastic, liquid or solid layer 30 as the case may be, all as fully described below.

In the present invention, shotgun pellets 25 are surface-

treated to impart a thin layer or film of material 30 which renders the pellets non-adherent by preventing metal to metal contact, and which may also inhibit or reduce the tendency of the shot to oxidize. This film 30 produced by surface-treating the pellets, has sufficient lubricating ability to permit the pellets to roll or slide easily over each other without adhering or sticking together. I am aware that it is very old to pour tallow, wax, or grease onto pellets in the shot charge, but the purpose of such practice is to increase the tendency of the shot to stick together and thereby obtain a very close or narrow pattern at the target, rather than to obtain an even distribution of the pellets over a larger area, as is obtained by my invention. It is, of course, the purpose of the choke 8 of the gun 7 to likewise obtain a very close or dense pattern, but it does this by causing a relatively high concentration in the center of the pattern and a relatively less even distribution through the pattern than is obtained by my invention.

Owing to the unreliability of the tallow, wax, or grease treatment, it has never been widely practiced. The tallow, wax, or grease filled the interstices between the pellets more or less completely, and added considerably to the weight of the shot charge. I am also aware that it has been proposed in U. S. Patent 189,417 to fill the interstices between the pellets with finely-divided solid material. My invention differs from these prior practices in that I use the very limited amount found necessary to surface-treat the pellets with material capable of preventing sticking and scuffing of the shot surfaces. Such treatment adds only a very small fraction of a percent to the weight of the shot charge. I am also aware that pellets have been copper coated, but I have found that copper-coated pellets tend to produce poorer patterns than shot which has not been copper coated. However, copper-coated shot obtained on the market produced better patterns when surface-treated by my invention.

Finely-divided, solid, non-sticking lubricating agents may be used to surface-treat the pellets by shaking or tumbling the pellets with the solid material. It is sometimes desirable to add an excess of the solid material and subsequently remove the excess by means of sieves, with blasts of air or the like. Materials which appear to be particularly applicable in my invention are powdered graphite and molybdenum disulfide, the latter being sold under the trade name of "Molykote." Other materials which are less effective but which give improvement in some cases are talc and powdered laminar materials, such as mica. Liquid high-pressure surface-lubricants may be applied by the agitation by the mixture of pellets and the liquid or by spraying the liquid onto the shot surface. Any material 30 which will give a tough non-metallic film of lubricating quality between the metallic surfaces 25 of the pellets 23 is satisfactory.

High-pressure lubricating oil additives were found valuable as the film 30 on the shot 23 in the present invention and were applied to the surface 25 of shot in the following manner: Shotgun shells were purchased in the open market. The shot charge from each shotgun shell was poured into a 100 cc. Florence flask, and two drops of the high-pressure lubricating oil additive were dropped onto the surface of the shot, which were then shaken by rotating the flask until the shot appeared to be covered with a uniform liquid film. Incidentally, one drop would probably have been sufficient. If too much surface-treating material is added to the shot, an undesirable amount of smoke will be noticeable when the charge is fired from the shotgun. After treating the shot charge as described above, the entire shot charge was returned to the shell and the crimp of the shotgun shell was restored. These high-pressure lubricating oil additives are so called because they give ordinary lubricating oil the power to resist high pressure and still lubricate. In addition, some of these have anti-oxidizing, and other valuable properties.

An alloy of 99.8% lead and 0.2% arsenic; or lead with small amounts of antimony and/or arsenic, or similar alloys, are used in the metallic portion 25 of the shot of the prior art, and such shot may be used in the present invention. However, the shot may be composed of any other suitable metals or alloys.

While poisonous materials can be used in my invention so far as the effectiveness of the shotgun pattern is concerned, the use of such materials is not recommended when game animals are killed for food. Such poisonous materials giving satisfactory surface-treatment to the pellets may be used at target practice, such as in skeet and trap shooting.

Another method for use with lead shot 25 is to treat the shot with chemicals which form a layer 30 of lead sulfate, lead chromate, lead chloride, or lead sulfide on the surface, which layer tends to protect the lead shot from oxidation.

In my invention I may also apply a thin film 30 of uncured phenolformaldehyde resin to the shot pellets and cure the film in place. I may also use urea formaldehyde or melamine resins cured in place as films on the surface of the shot pellets. I may also apply regenerated cellulose or cellophane film by applying a film of viscose and passing the shot separately through a suitable regenerating jet. The usual plasticizers and other compounding agents known to those skilled in the art may be used in compounding and applying these resin films to the shot.

#### Example

In order to test the present invention, a number of shotgun shells were fired from the same 12 gauge gun having a 26-inch improved cylinder barrel at paper targets placed at a distance of 40 yards. A 30-inch circle was then located on each target so as to include the maximum number of perforations made by the individual pellets. After said 30-inch diameter circle is so located, then the target is studied to see how many five-inch diameter circles can be drawn, which five-inch circles do not intersect each other, do not surround any shot perforation, and yet lie entirely inside said 30-inch circle. Each such unperforated five-inch circular area is known to those skilled in the art as a five-inch patch, the area being just that which could be occupied by a duck or similar sized game bird or animal, within said 30-inch circle, without said duck being immediately killed by the shot pellets. Obviously the larger the number of five-inch patches in a pattern, the poorer the shotgun shell, and the more game animals that escape unharmed or in a crippled or slightly wounded condition. Other size patches could be selected for calculations involving other size game, but five-inch patches are representative and about the average size for game hunted with a 12-gauge shotgun and No. 6 shot. The shotgun shells were all 12-gauge shells containing 1.25 ounces of No. 6 shot from the same lot of the same manufacturer. The opening of the individual shells was made very carefully, and all the shells were opened and reassembled after the surface treatment of the shot. The control shell, likewise, was opened, the number of pellets counted, and those pellets returned to the control shell, omitting the surface-treatment. The following comparative results were obtained with the surface-treated pellets as compared with the untreated pellets:

| Test No. | Surface-Treating Material               | No. of 5" Patches | Reduction in Patchiness, percent | Remarks                         |
|----------|-----------------------------------------|-------------------|----------------------------------|---------------------------------|
| 1.....   | None.....                               | 10.....           | .....                            | This cartridge used as control. |
| 2.....   | Graphite.....                           | 5.....            | 50.....                          |                                 |
| 3.....   | High-pressure lubricating oil additive. | 5.....            | 50.....                          |                                 |

The particular high-pressure lubricating oil additive used in the above test was "Lubrizol 1851C" which comprises a barium salt of a substituted phenol-formaldehyde condensate. This material in addition to its high-pressure lubricating values has anti-oxidizing and other similar valuable qualities in lubricating oil, and these same qualities add to its value in the present invention. Other high-pressure lubricating oil additives give valuable results in the practice of the present invention as the film on the shot.

While preferred embodiments of the invention have been disclosed for the purpose of illustration the invention is not limited thereto but is defined in scope by the following claims.

I claim as my invention:

1. A shotgun cartridge characterized by having a projectile charge of metallic shot pellets coated with a coating consisting essentially of barium salts of substituted phenol-formaldehyde condensate, said coating being sufficiently thick to inhibit oxidation, metal to metal contact and welding and sticking together of said pellets under the pressure of the explosion of said shotgun cartridge.

2. Shot for use in shotguns comprising metal pellets coated with a coating consisting essentially of barium salts of substituted phenol-formaldehyde condensate, said coating being sufficiently thick to inhibit oxidation, metal to metal contact and welding and sticking together of the pellets during use.

3. A shotgun cartridge characterized by having a projectile charge of metallic shot pellets coated with an oxidation inhibiting, metal to metal contact inhibiting film of a non-metallic material comprising barium salts of substituted phenol-formaldehyde condensate of sufficient thickness whereby metal to metal contact of the pellets is prevented during the firing of the shotgun cartridge and the tendency of the shot to cling together during its passage through the shotgun is substantially reduced.

4. Shot for use in shotguns comprising metal pellets coated with an oxidation inhibiting, metal to metal contact inhibiting film of a non-metallic material comprising barium salts of substituted phenol-formaldehyde condensate of sufficient thickness whereby metal to metal contact is prevented and the tendency of the shot to cling together in use is substantially reduced.

References Cited in the file of this patent

UNITED STATES PATENTS

|           |         |               |
|-----------|---------|---------------|
| 204,298   | Crooke  | May 28, 1878  |
| 207,582   | Wright  | Aug. 27, 1878 |
| 573,120   | Wheeler | Dec. 15, 1896 |
| 2,579,329 | Martin  | Dec. 18, 1951 |

FOREIGN PATENTS

|         |               |               |
|---------|---------------|---------------|
| 8,820   | Great Britain | of 1913       |
| 498,923 | Great Britain | Jan. 11, 1939 |